

## UNITED STATES PATENT OFFICE.

MEINRAD F. THOMA, OF FITCHEBURG, MASSACHUSETTS.

## PROCESS OF MIXING SILK AND ARTIFICIAL SILK.

No Drawing. Application filed March 2, 1927, Serial No. 172,203. Renewed June 14, 1928.

This invention relates to the production of a fabric from a mixture of animal and vegetable fibers, e. g. natural and artificial silk fibers.

5 The principal object of the invention is to mix the two kinds of fibers before they are spun or even in condition for spinning, so that the fibers themselves are intimately intermingled in the resulting yarn in such a way 10 as to bring out a cross dye effect when the product is dyed.

The invention has for one of its advantages the fact that woven fabric can be manufactured from the mixed fibers of the two kinds 15 and dyed after it is woven, the dye taking effect evenly on the two kinds of fibers and producing new and beautiful effects on account of the fact that the individual fibers with the separate effects are so finely intermingled.

Another object of the invention is to provide for changing the relative length of the fibers by introducing the step of breaking the long fibered natural silk while it is intermingled with and surrounded by the shorter fibered artificial silk, in such a way that the silk fiber will retain its position in the stock and be held in place by the artificial silk which surrounds it and prevents its being 30 materially displaced in the sliver in which it is located and to accomplish this without danger of breaking the artificial silk fibers.

Other objects and advantages of the invention will appear hereinafter.

35 As stated, this invention relates to the mixing of two kinds of fiber. It is well known that real silk and artificial silk do not take colors in dyeing in just the same way. Some colors the artificial silk does not take at all, 40 while in the same dye the real silk will be colored perfectly. I take advantage of that fact in this process to produce a yarn not made up of twisted fibers of artificial silk combined with twisted fibers of real silk, but 45 made up with an intermingling of the two kinds of fiber in their early stage of manufacture before they approach the form of yarn in any way.

On account of this intimate and minute 50 mixture, the yarn produced can be woven in any ordinary way and subjected to dyeing. The dyeing will have the same effect on each individual fiber as it would if the cloth were made entirely of that, but the effect on the 55 cloth is very materially changed. Different

shades and even different colors are imparted to the two kinds of fibers in the same vat, and the result is not a mixture of the two shades or colors in the ordinary sense: that is, they cannot be distinguished from each other in 60 the fabric, but the result is different from either one. This is an important advantage of the invention.

In carrying out the invention, I put into a carding machine a mixture of real silk, as for 65 example, in the form of schappe, and artificial stable fiber in whatever proportion may be desired, as for example, 40% of real silk and 60% of artificial silk or one part silk to two parts artificial silk. These fabrics are 70 operated upon in the usual way and produce a sliver which consists of two kinds of fibers mixed intimately together, and of comparatively uniform appearance throughout. Ordinarily the artificial silk is in lengths of ap- 75 proximately an inch and a half while the schappe silk, if that is used, is in lengths of four inches or thereabout.

Such a combination cannot be spun, and for that purpose I introduce the lap into a 80 breaking machine which consists of two pairs of rolls supported at a distance apart equal to or greater than the length of the artificial silk fiber, whatever that may be, and run the front rolls faster than the rear rolls. 85 For safety an additional pair of rolls can be used having the same relationship to the first pair as that has to the other. The result of this is that the commingled fibers are subjected to a pulling action between the 90 rolls of adjacent pairs, but this pulling action can have no effect on the artificial silk fibers because they are not long enough to have both ends in the bight of the two pairs or rolls at the same time. On the contrary 95 the real silk fibers are long enough and they are broken apart by the pull, but when they are broken apart they are surrounded by and intermingled with artificial silk to such an extent that they cannot crinkle up and contract, and they are carried along in an uninterrupted manner throughout the process.

100 This sliver is then passed through other machinery, such as is commonly used in the silk industry or even in the cotton industry, and finally through any desired kind of a spinning machine and spun into uniform 105 yarn from which either the warp or the weft, or both, of a fabric can be made. This fabric, as stated, is capable of being dyed in the 110

manner specified, and novel and beautiful results are obtained from it.

Although I have described a particular method of carrying out the process of subjecting the two kinds of fiber to the several processes necessarily involved and the particular order of steps, I am aware of the fact that some changes can be made in the order and number of steps employed without departing from the scope of the invention as expressed in the claims. Therefore, I do not wish to be limited in these respects, but

What I do claim is:—

1. The method of making a fabric which consists in mixing about one part of schappe silk with two parts of artificial silk, carding the mixture, breaking the schappe silk fibers when surrounded by artificial silk fibers, spinning the mixture, weaving the yarn, and

20 dyeing it in the piece.

2. The method of preparing yarn for spinning, which consists in mixing short artificial silk fibers with longer natural silk fibers, carding the mixture and producing there-

25 from a sliver, subjecting the sliver to a draw-

ing action in which the points at which the sliver is gripped are farther apart than the length of the artificial silk fibers but less than that of the natural silk fibers, so as to break the natural silk fibers without breaking the 30 artificial silk fibers, and thereafter spinning the product.

3. As a new product a composite yarn consisting of intimately intermingled schappe silk fibers and short artificial silk fibers, in 35 which the schappe silk fibers have been broken when surrounded by the artificial silk fibers in the sliver to a length not greater than the length of the artificial silk fibers.

4. As a new product a composite yarn consisting of intimately intermingled natural silk fibers and short artificial silk fibers, in which the natural silk fibers have been broken when surrounded by artificial silk fibers in the sliver to a length not greater than the 40 length of the artificial silk fibers.

In testimony whereof I have hereunto affixed my signature.

MEINRAD F. THOMA.